

## UNITED STATES PATENT OFFICE

JAMES BADDILEY, OF BLACKLEY, MANCHESTER, ENGLAND, ASSIGNOR TO BRITISH DYESTUFFS CORPORATION LIMITED, OF MANCHESTER, ENGLAND

## PROCESS OF DYEING

No Drawing. Application filed May 26, 1927, Serial No. 194,542, and in Great Britain September 7, 1928. Divided and this application filed December 11, 1928. Serial No. 325,397. Renewed September 24, 1939.

In my co-pending application Serial No. 194,542, I have described the dyeing of regenerated cellulose silk, such as viscose silk, in level shades, with the monoazo dyestuffs obtained on coupling diazotized aromatic amines, their homologues, derivatives, and the sulphonic acids and carboxylic acids thereof with a 2-amino-5-naphthol-7-sulphonic acid, including in this expression its N-substituted derivatives. Some of the dyestuffs of this class are already known but they have never been used commercially, probably because they possess too small an affinity for cotton.

It is stated in the above mentioned application that I have made the entirely unexpected discovery that these dyestuffs possess a good affinity for regenerated cellulose silks and in particular that they give level dyeings on these fibres. It is now well known that the regenerated cellulose silks generally possess a very uneven avidity for the usual cotton colours, which causes the dyeings obtained to be unlevel. My discovery of a range of dyestuffs which give even dyeings on these fibres is therefore of considerable value to those engaged in the process of dyeing regenerated cellulose silks.

Among the dyes included in the above, I have found that the monoazo dyestuff obtained by coupling diazotized aniline with a benzoylated 2:amino-5-naphthol-7-sulphonic acid gives particularly very even dyeings on regenerated cellulose silk. In the above example in place of aniline, there may be substituted beta-naphthylamine, para-nitroaniline, meta-aminobenzoic acid, 2-naphthylamine-6:8-disulphonic acid and para-chloroaniline, the dyestuffs obtained being especially valuable in producing level shades in dyeings on regenerated cellulose silk. These aryl amines have the general formula  $H_2N-R_2$  wherein  $R_2$  represents a phenyl or naphthyl residue or the nitro, chloro, sulphonic or carboxylic derivatives of such residue.

The regenerated cellulose silk materials are dyed in the usual way. The following description is typical of the manner in which the dyeing may be carried out, but it must be

understood that these conditions may be varied considerably and that I do not limit myself to the conditions given in the example.

*Example.*—The dyebath is made up from 3,000 parts of water and 1 part of the dyestuff produced by combining the diazo compound of aniline with benzoyl-2-amino-5-naphthol-7-sulphonic acid. 100 parts of the regenerated cellulose silk material are entered into the dyebath, which is then brought to the boil. About 10 parts of Glaubers' salt or common salt are then added and dyeing allowed to proceed at or near the boil for  $\frac{1}{2}$ - $\frac{3}{4}$  hour. If desired soap may be added to the dyebath. The fabric is dyed a bright red shade, the dyeing being particularly level.

What I claim and desire to secure by Letters Patent is:—

1. A process of dyeing regenerated cellulose material in level shades, characterized by the application to the material of a monoazo dyestuff obtained by coupling a benzoylated 2-amino-5-naphthol-7-sulphonic acid with diazotized aniline.

2. The process of dyeing regenerated cellulose material in level shades characterized by the application to the material of monoazo dyestuffs obtained in coupling benzoylated 2-amino-5-naphthol-7-sulphonic acid with a diazo compound.

3. The process of dyeing regenerated cellulose material in level shades characterized by the application to the material of a monoazo dyestuff obtained by coupling benzoylated 2-amino-5-naphthol-7-sulphonic acid with a diazotized aryl amine having the general formula  $H_2N-R_2$  wherein  $R_2$  represents a phenyl or naphthyl residue or the nitro, chloro, sulphonic or carboxylic derivatives of such residue.

In witness whereof I affix my signature.  
JAMES BADDILEY.